

Dec. 14, 1937.

K. F. WHITCOMB ET AL

2,102,343

GRINDING WHEEL

Filed July 3, 1933



FIG. 4

FIG. 5



FIG. 3



FIG. 2



FIG. 1

KENNETH F. WHITCOMB  
HERBERT W. WAGNER

By *Clayton L. Jenke*  
Attorney

## UNITED STATES PATENT OFFICE

2,102,343

## GRINDING WHEEL

Kenneth F. Whitcomb and Herbert W. Wagner,  
Worcester, Mass., assignors to Norton Com-  
pany, Worcester, Mass., a corporation of  
Massachusetts

Application July 3, 1933, Serial No. 678,816

13 Claims. (CL 51—206)

This invention relates to a grinding wheel, and particularly to that type of wheel which is made of abrasive grains united into an integral body by a suitable bond, such as rubber, shellac, the 5 resinoids, sodium silicate and vitrified ceramic materials.

The primary object of this invention is to provide a grinding wheel of standard grinding characteristics and of uniform structure 10 throughout its effective grinding zone, but which is so reinforced that it may be rotated at a rapid rate or used under severe temperature conditions without breaking, and which will serve with high efficiency in a grinding operation. Other objects 15 will be apparent in the following disclosure.

The two major destructive forces which tend to break a grinding wheel are the centrifugal force due to rotation of the wheel and the stress set up by differential temperatures in the wheel 20 resulting from the heat of grinding on its periphery. These influences build up their most destructive effects adjacent to and around the central hole of the wheel. This invention, therefore, contemplates fortifying the wheel against 25 breakage by making the inner zone or central portion of the wheel around the hole more resistant to these forces than is the grinding zone of the wheel, whose properties are fixed by the grinding characteristics required for a given 30 operation. Such a grinding wheel may comprise at least two zones, an outer annulus which serves for the grinding operation, and an inner zone adjacent to the arbor hole which is more resistant to the sum of the two stresses than is the 35 material of the grinding zone, or to that stress which is predominant and tends to cause breakage of the wheel.

In the drawing:

Fig. 1 is a set of curves illustrating certain 40 stresses in a grinding wheel shown in Fig. 2;

Fig. 2 is a section through a composite two- 45 zone wheel, arranged to correspond with the curves of Fig. 1;

Fig. 3 is a plan view of the wheel;

Fig. 4 is a detail of the joint between the two 45 zones; and

Fig. 5 illustrates a mold for shaping a two-zone wheel.

In this multiple zone wheel, the outer grinding 50 zone must be made in accordance with the desired grinding characteristics, as regards the nature and kind of the abrasive, the grain size, the nature, type and quantity of the bond, the volume percentages of the abrasive, bond and pores, the wheel dimensions and uniformity of

thickness and other fixed characteristics of the wheel. Hence, this outer zone structure cannot be changed. It is, therefore, desirable that the characteristics of the inner strengthening zone of the grinding wheel be so selected as to meet 5 the various requirements determined by the conditions under which the wheel is to be manufactured and used, so as to prevent cracking or a strained condition at the joint and to strengthen and form an integral body with the outer 10 zone. In the manufacture of a vitrified grinding wheel, the requirements of the average manufacturing operation indicate the desirability of having the same bond and type of grain in the two zones, so that the wheel may be easily manufactured as a unit; but if desired, and within the scope of this invention, the two zones may be made of radically different materials, provided all or the more important of the fundamental 15 conditions outlined below are satisfied. For example, a vitrified wheel may be provided with a rubber or a synthetic resinoid center, with or without abrasive material therein, as hereinafter explained. Likewise, other wheels may be strengthened by means of centers which are 20 adapted for the purpose. The invention will, however, be described specifically with reference to the manufacture of a ceramic bonded wheel in which the bond in each zone is a ceramic material capable of being vitrified to a glassy or porcelainic condition in the presence of the 25 abrasive grains.

## Strength of wheel structure

The strength of the wheel structure depends 35 upon the grain size and the quantity and type of bond and grain employed. As the grain size decreases, the strength increases within certain limits, if the volume structure of the wheel remains the same. However, after the grain size 40 has been decreased to a certain point, the maximum strength per unit of volume is obtained. Experimental work has developed the fact that this maximum strength of a ceramic bonded article is approached when the grain particles have been reduced to approximately that size at which the grains will just pass through a screen of 100 meshes to the linear inch or somewhat finer. Therefore, the inner zone may be strengthened 50 by using a finer grain size than found in the outer zone, and preferably as fine as 100 mesh. Coarse grains may be interspersed with the fine grains, but a considerable amount of the grains should be fine. It is also possible to increase the strength of the inner zone by the use of more 55

bond or a bond of greater intrinsic strength, provided it will unite integrally with the material of the outer zone. The wheel structure may be strengthened, therefore, by:

- 5 (1) Employing a finer size of grain in the central zone than is used in the grinding zone, and preferably while maintaining the same volume percentage of abrasive in the two zones.
- 10 (2) Using the same grain size and the same volume percentage of bond in the two zones, but having a greater amount or volume percentage of grain in the inner than in the grinding zone.
- 15 (3) Having a higher bond volume percentage in the inner than in the outer zone.
- 20 (4) Using a bond in the inner zone which has a higher intrinsic strength than that used in the outer zone.
- (5) Employing a combination of the above features.

#### Relative sizes of the two zones

A further factor which should be considered is the ratio of the diameter of the reinforcing or inner zone to that of the outer grinding zone. 25 It is desirable that the reinforcing inner zone be as large as practicable. The ideal wheel is one in which the material of the inner zone is so selected that, as the stress in the outer zone at the edge of the joint approaches the ultimate 30 strength of the outer zone material, the inner zone is of such strength and size that, although it has strengthened the wheel, it will break just before the outer zone breaks, and this break will start at the edge of the hole.

35 Fig. 1 shows a typical stress distribution in a standard grinding wheel of a given structure, illustrated in Fig. 2 in correct relationship to the curves, which has a radius of 12" and a small hole of 1" radius. As there plotted, it will be 40 apparent that the tangential stress due to rotating the wheel at a high speed and the stress set up by the frictional heat of grinding are very high at the edge of the hole 10, indicated by the line *a* in Fig. 1, and that the major portion of this 45 stress is found within a short distance of the center of the wheel. It will, therefore, be appreciated that the inner zone of the wheel need not extend radially outwardly beyond that point at which the stresses have become comparatively 50 small. In such a wheel, an inner zone having a radius equal to one-third of the radius of the wheel body, i. e., the distance from the edge of the hole to the periphery of the wheel, will be subjected to the major portion of the disruptive 55 forces met in a grinding operation, as indicated by the line *b* in Fig. 1, which corresponds with the position of the joint 11 between the outer zone 12 and the inner zone 13 of the wheel shown in Figs. 2 and 3. This inner zone may be made 60 larger or smaller, proportionate to the outer zone, as determined by the particular characteristics of the grinding wheel under consideration, but ordinarily it should not make up more than half of the radial thickness of the wheel. 65 In particular, the inner zone should not extend into that space normally assigned for grinding use, and it is preferable that it lie wholly within the outer edges of the flanges or plates which support the grinding wheel on the spindle.

#### Requirements at the joint between the zones

To make this invention practical, certain requirements at the joint or circular junction of the two zones must be taken into account in order that separation of the bodies of the two zones

may be prevented, as well as creation of a high stress in either body adjacent to the joint.

The volume changes which cannot be prevented and must be provided for are both permanent and reversible. The permanent change 5 is caused by shrinkage when the bond is dried and matured. The reversible changes are caused by cooling the bond after it has been matured and by the stretching of the wheel during grinding due to centrifugal force and frictional heat. 10 When a volume change occurs in the material of one zone at or near the joint, approximately the same volume change should occur in the adjacent portion of the other zone. To accomplish this matching of the volume changes, the bodies of the two zones in an ideal wheel should have approximately equal values for each of the following properties, as explained below:

(1) Shrinkage due to drying and maturing the bond during manufacture of the wheel 20

(2) Coefficient of thermal expansion of the body during manufacture and use

(3) Modulus of elasticity during manufacture and use of the wheel.

If the properties (1) and (2) are not near enough equal, one zone will be subjected to a stress tending to produce a crack between the two zones. In regard to the third property, a deformation of body set up at the joint, by centrifugal force or differential heating, will deform the materials of both zones at the joint. If the modulus of elasticity of the inner zone is much higher than that of the outer zone, the outer zone material, being less stiff, will accommodate more than its share of the required deformation, and tend to reach its breaking point too soon, which would result in premature failure of the wheel.

#### Shrinkage during drying and maturing the bond 40

As above stated, it is desirable that the drying and firing shrinkages of the two portions be equal or so matched that the parts will remain in proper relation to one another, during use as well as manufacture of the wheel. Some of the 45 factors to be considered are:

(1) The volume percentages of abrasive and of bond in both zones while in the green unfired stage;

(2) The kind of abrasive and its size and shape and the kind of bond in each zone;

(3) The amount of removable constituents, such as water or other plasticizer required to make a moldable mixture of the grains and bond; and

(4) The variations in heat treatments and maturing temperatures of the bond, so that two zones may be formed at the same time.

An ideal composite wheel is one where the drying and firing shrinkages of the outer and inner zones are the same. Some differential shrinkage is permissible if the strengths of the two materials are sufficient to prevent rupture although a strained condition is set up. It, however, is necessary to select the proper materials for the inner zone so that its characteristics will match those of the outer zone which cannot be changed.

#### Coefficients of expansion 70

In the manufacture of a vitrified wheel, in which the vitrifiable ceramic material is fired to a fluid condition and then solidified, it is necessary that the two zones of material contract at substantially the same rate during the 75

cooling of the bond after it has become hard. The same considerations apply, of course, to any heating up of the wheel during its storage or use. The coefficients of expansion of the bond and the individual grains should preferably satisfy the conditions set forth in the Patent to Saunders, Milligan and Beecher No. 1,829,761, dated November 3, 1931. The present considerations, however, apply to the substance of each zone taken as a whole and refer particularly to the joint along which the materials of the two zones lie in contact. It is necessary that the inner zone shall not contract more rapidly than the outer zone and thus pull away from it. On the other hand, the outer zone should not shrink more than does the inner zone and to such an extent as to set up strains within the outer zone which will tend to rupture it, during either the cooling operation or the subsequent use of the wheel. It will, therefore, be appreciated that while the ideal conditions are not always practical, it is satisfactory to have the coefficients of expansion of the two zones so nearly alike within the elastic limits of the materials that the wheel will not rupture during manufacture or use and that strains will not be set up in either of the zones which are sufficient to cause such rupture at any time during the life of the wheel.

#### Modulus of elasticity

The modulus of elasticity may be defined as the ratio of the stress applied at rupture of the wheel to the percentage of elongation produced by that force, and it is a measure of the stiffness or resistance to distortion of the material.

The ideal composite grinding wheel is one in which the structures of the two zones are such that their moduli of elasticity are substantially equal, or as nearly equal as the other factors permit. However, it is found that the modulus of elasticity of either zone of a vitrified wheel may be as much as 2.6 times as great as that of the other zone; but it is preferable that the modulus of elasticity be the greater in the outer zone if equality is not feasible. In such a case, the outer zone would have the greater stiffness, and the inner zone would have the greater ability to stretch under the forces applied to the wheel by rotation and heat applied at the periphery. This theoretical value, which is subject to experimental error, may be departed from widely because of other considerations which may control the manufacture of the wheel; and a reasonable latitude of interpretation of the claims is, therefore, to be had.

#### Ability of the inner zone to stretch

As to the ability of the inner zone to stretch tangentially at the edge of the hole without breaking, when subjected to either centrifugal force or differential temperatures, the following considerations are to be noted. In the ideal wheel, the deformation at rupture of the inner zone should be greater than that of the other zone, in order to resist heat breakage. In other words, where the two zones have the same moduli of elasticity, the inner zone will have the greater strength and the greater deformation at rupture, as indicated by Equation (1). That is, if the inner zone has twice the strength but the same modulus of elasticity as has the outer zone, then it can stretch twice as much at the edge of the hole at rupture as would a wheel made wholly of the outer zone material. Since the moduli are the same, the material on each side of the joint will stretch the

same, although one is stronger than the other, and the wheel cannot pull apart laterally at the joint. If two different grinding wheels have the same tensile strengths, but different values for deformation at rupture, they will have unequal resistance to heat breakage; and that wheel which has the greater ability to stretch will withstand the higher temperature difference. For example, an organic bonded grinding wheel, such as one made of crystalline alumina grains bonded by means of a synthetic resinoid (e. g., a heat-set phenolic aldehyde condensation product), may have the same tensile strength as a grinding wheel made up of the same abrasive grains bonded by a vitrified ceramic material; but because of the fact that the resinoid has the higher value for its deformation at rupture, it will stand greater temperature differences between the periphery and the center. On the other hand, it will be appreciated that a mere ability to stretch is insufficient to withstand centrifugal stresses, since an inner zone of soft rubber could not strengthen the wheel. The material must have both stiffness and strength to resist breakage in use.

#### Compositions and structures of composite wheels

In accordance with this invention, it is proposed to make composite grinding wheels which satisfy the major conditions above set forth, and preferably all of them. To manufacture such wheels successfully and on a commercial basis, it is necessary that the structures of the two or more zones in the composite wheel shall have such physical properties and bear such relationship to each other as to avoid a strained condition at the joints between the various zones of the wheel; and the wheel structures should be so constituted that these properties remain constant throughout the life of the wheel. It is, therefore, desirable in accordance with this invention to employ what is known as the controlled structure method of manufacturing such a wheel, as fully set forth in the patent to Wallace L. Howe and Richard H. Martin, No. 1,983,082, dated December 4, 1934, and the British Patent No. 385,328. In accordance with that procedure, the volume percentages of the granular material, the bond and the pores of the final product are accurately precalculated to give the desired wheel characteristics. This procedure comprises determining the volume which the granular material and the bond will occupy in the final product in each of the zones, taking into account the shrinkages involved in molding and shaping and drying the wheel and later in maturing the bond, such as is involved in firing a mixture of ceramic materials to vitrify the same. The next step, based on these precalculations, is to determine that volume which the raw materials in intimate mixture shall occupy in the mold while in a green condition, so that when the bond has been matured, the body of each zone will shrink to the precalculated volume. The operation of causing this molded mass of green material to occupy the required volume in the raw condition may be accomplished in various ways, such as by jolting the mixture in a mold on a suitable jolting machine, or preferably by pressing the green mass in a mold of accurate dimensions to the required volume, but without any regard to the shape of the grains or the degree of pressure required. This controlled structure method may be employed for the different types of bond, as will be readily understood. Ceramic materials of any desired formulas, or which are of standard compositions, may be used

for forming a vitrified bond, and the abrasive materials may be silicon carbide, crystalline alumina or any other suitable abrasive. Such a ceramic mixture with the abrasive grains of required size and in amounts which have been precalculated to give a desired structure in the outer grinding zone will be intimately mixed with a slight amount of a plasticizing medium, such as water, and this slightly moistened mass is then ready to be molded in the press. Similarly, the volume structure of the inner zone will have been precalculated, and the granular material and bond therefor measured in accordance with these calculations. In this inner zone, one may use either the same abrasive material as employed in the outer zone or, if desired, any suitable granular material, and preferably substances which are not expensive but will satisfy the conditions set forth above. It is feasible to employ either the same general type of bond as used in the outer zone, or one may use altogether different bonds. For example, if the outer zone bond is a vitrifiable ceramic material, the inner zone may be made of a similar or different ceramic materials, or it may be made of rubber, the artificial resinoids or other materials, with or without abrasive grains or fillers, and which are standard bonds in this art and need not be fully described herein. A vitrifiable ceramic material may also be used alone without any granular material for the inner zone, provided the characteristics of the porcelain or glass satisfy the above conditions.

Various expedients may be employed which will aid in uniting the materials of the two zones. It, for example, is feasible to employ a lapped joint, as illustrated in Fig. 4, in which case the joint between the two zones is staggered so that teeth, as it were, on each of the zones will interlock with and project into the material of the other zone and contact intimately therewith.

As a simple illustration of a structure which is suitable for the purpose of molding these two zones, reference is to be had to Fig. 5 of the drawing. As there shown, a mold cylinder 20 of suitable internal dimensions may be placed on a mold plate 21, and a cylinder 22 of required dimensions to provide the inner zone is placed therein. This inner cylinder 22 is short, as illustrated, and is spaced from the mold plate 21. This may be accomplished by providing the inner cylinder with four radial strips 24 of equal length, which are spaced around the outside of this cylinder 22 and are integrally joined thereto. These serve to hold the inner mold in its correct position. These four equally spaced small strips are set upon wooden blocks 25 of approximately 1" thickness.

Having now arranged the parts in this fashion, the mixture of material 26 for the inner zone is then poured into the inner cylinder 22 to a depth of about 1", and it will flow under the edges of the cylinder until it reaches the angle of repose. Then, the outer zone material is poured into the annular space around the inner ring to a depth of about 1", thus covering the inner zone material that has spread out under the inner mold wall. The inner cylinder is then moved upwardly for a short distance, and the operation repeated. These steps are done successively until the outer mold has been filled with the material, as required. This method results in the zigzag joint shown in Fig. 4.

Following this operation, a cover plate is placed within the mold 20 and subjected to pressure to compact the material and squeeze the pores

to such an extent that the two zones are compelled to occupy that total volume which has been precalculated for the wheel of this particular structure. Thereafter, the molded material is removed from or left in the mold, depending upon the final bond maturing operation, and the bond is matured. In the case of a ceramic bonded wheel, the wheel is removed from the mold and properly dried, and then placed in a suitable kiln and heated to a vitrifying temperature as required for the particular bond being used which, for the standard vitrifiable bonds, is ordinarily from Seger cones 4 to 13. In the case of a resinoid or rubber bond, the material may be left in the mold and there heat treated under pressure or as desired to heat-set the bond. Such bonds may be matured in accordance with the standard methods.

#### Wheel compositions

It will be apparent, in view of the above statements, that grinding wheels will differ materially in their compositions and structures and that consequently the composition of the inner zone of each wheel will necessarily be determined by the composition and structure of the outer zone. As an example of one particular composition and structure, we may assume that a particular grinding operation requires a wheel of 24" diameter, 2" thickness and 2" hole. The grain size in the grinding zone may be such as will just pass through an 18 mesh screen and be designated 20 mesh. This wheel may be made of either silicon carbide or crystalline alumina abrasives and bonded by suitable materials. In the present instance, crystalline alumina abrasive and a ceramic bond are chosen. A suitable bond may have the following composition:

|                                |       |    |
|--------------------------------|-------|----|
| SiO <sub>2</sub>               | 55.0  | 40 |
| Al <sub>2</sub> O <sub>3</sub> | 11.4  |    |
| Fe <sub>2</sub> O <sub>3</sub> | 4.3   |    |
| MgO                            | 2.8   |    |
| CaO                            | 5.9   |    |
| Na <sub>2</sub> O              | 6.0   | 45 |
| K <sub>2</sub> O               | 2.6   |    |
| TiO <sub>2</sub>               | 0.7   |    |
| B <sub>2</sub> O <sub>3</sub>  | 11.3  |    |
|                                | 100.0 | 50 |

To obtain a desired grade of hardness, 25% ounces of the green ceramic bond mixture may be used per pound of crystalline alumina abrasive, together with sufficient water to render the mass moldable. The amount of abrasive and bond are so proportioned that the resultant grinding wheel will have 54% by volume of abrasive in the outer grinding zone. When this mixture of bond and grains has been vitrified in the ceramic kiln at a suitable firing temperature, the vitrified structure of the outer zone has approximately the following properties:

Modulus of elasticity =  $9.4 \times 10^6$  lbs. per sq. in.  
Tensile strength = 1900 lbs. per sq. in.  
Shrinkage (volumetric) = 0.9%  
Coefficient of expansion = 0.0000067 per degree centigrade.

The central zone is preferably so constituted that it has the same values for modulus of elasticity, shrinkage and coefficient of expansion, but has a greater strength, thus giving a greater deformation at rupture in the inner zone and thereby strengthening the wheel. The modulus of elasticity of the inner zone may be varied to be smaller than that of the outer portion, but

for the sake of making the two zones unite integrally without strain, it is desirable that they have the same coefficient of expansion and shrinkage. To this end, the inner zone mixture may be made of abrasive grain of 36 grit size; the structure may be one which has 52% by volume of abrasive; and 3 1/4 ounces of the same bond as used in the outer zone may be employed per pound of abrasive. This composition, when 10 fired, will have a tensile strength of 2900 lbs. per sq. in., as distinguished from the 1900 in the outer zone, thus producing a far stronger center zone than is the outer zone. If it is desired that the central zone be 12" in diameter or extend 15 half way radially outwardly, the proper amounts of the mixtures by volume and weight are proportioned as follows:

|                            | Outer zone  | Inner zone    |
|----------------------------|-------------|---------------|
| Zone size.....             | 24x2x12"    | 12x2x2"       |
| Volume of raw mixture..... | 699 cu. in. | 200.8 cu. in. |
| Weight of raw mixture..... | 64.3 lbs.   | 18.5 lbs.     |

After the wheel mixtures have been molded in the manner above described, and the mass vitrified in a ceramic kiln at approximately Orton cone #12, a unitary grinding wheel is thus made 30 which is far stronger than one made solely of the outer zone material, and which will stand a far higher rate of rotation and a temperature differential.

As a second example, a two-zone grinding wheel may be made in accordance with the following specifications:

#### Outer grinding zone

|                                                                      |                                                                |
|----------------------------------------------------------------------|----------------------------------------------------------------|
| Crystalline alumina abrasive.....                                    | 1/2 of 30 and 1/2 of 36 grit size                              |
| 40 Vitrifiable bond of the composition given in the above table..... | 3 1/2 ounces of bond per pound of crystalline alumina abrasive |
| Structure.....                                                       | 50% by volume of abrasive in the finished wheel                |
| Modulus of elasticity.....                                           | $8.8 \times 10^6$ lbs./sq. in.                                 |
| 45 Tensile strength.....                                             | 2650 lbs./sq. in.                                              |
| Shrinkage.....                                                       | 1.0%                                                           |
| Coefficient of expansion.....                                        | 0.0000067/deg. C.                                              |

#### Inner grinding zone

|                                                  |                                              |
|--------------------------------------------------|----------------------------------------------|
| 50 Crystalline alumina abrasive.....             | 1/2 of 60, 1/4 of 70 and 1/4 of 80 grit size |
| Vitrifiable bond, same as in the outer zone..... | 3 1/2 ozs. bond/lb. of abrasive              |
| Modulus of elasticity.....                       | $8.7 \times 10^6$ lbs./sq. in.               |
| Tensile strength.....                            | 3800 lbs./sq. in.                            |
| Shrinkage.....                                   | 1.0%                                         |
| 55 Coefficient of expansion.....                 | 0.0000067/deg. C.                            |

#### Proportions in completed wheel

|                        | Outer zone     | Inner zone    |
|------------------------|----------------|---------------|
| 60 Zone size.....      | 30 x 3 x 15"   | 15 x 3 x 3"   |
| Volumes.....           | 1564.5 cu. in. | 511.2 cu. in. |
| Weight of mixture..... | 141.6 lbs.     | 45.0 lbs.     |

65 A grinding wheel may have a center of other material capable of increasing its strength and resistance to ruptural deformation. For example, a vitrified grinding wheel may be provided with a center of a synthetic resinoid which will mold easily and not shrink detrimentally. A suitable material for the purpose is a hot molding compound of wood flour and "Bakelite" resinoid, which is a standard compound on the market. This compound may be molded in a soft condition around an arbor in the center hole of a 70

previously fashioned vitrified wheel and then be set to a hard condition by a combination of heat and hydraulic pressure, as is well known in the art. The center of the vitrified wheel may be initially painted with a suitable solution of the resinoid so as to promote penetration of the inner zone material into the pores of the vitrified body and its adhesion thereto. The resinoid may include other fillers, such as quartz, which serve to strengthen it or otherwise improve its properties, such as by cutting down the shrinkage of the material when it is hardened. Abrasive material, and particularly the fine sizes, may be used with the resinoid in accordance with the principles outlined above. 10 15

Similarly, a grinding wheel, such as a vitrified wheel as above described, may be strengthened by a hard rubber center. As an example, a grinding wheel may be made according to standard procedure of abrasive grains bonded by a vitrified ceramic material, but with the hole of a suitable oversize. Within this hole, a strip of rubber compound capable of vulcanizing to a hard condition is placed in contact with the peripheral surface of the wheel hole and then a suitable rubber compound, such as a mixture of one part by weight of rubber to seven of abrasive grains, is placed between the strip and an arbor of desired diameter. The abrasive may be crystalline alumina or other material, and preferably of a fine size, such as 60 grit or finer. The rubber compounds are made in accordance with standard procedure, and they are used in such amounts that when pressed, they will fill the space between the arbor and the surface of the 20 25 30 35

45 wheel hole. By heating the rubber, while applying pressure thereto, the rubber strip is forced to flow into the wheel pores to a desired extent. Further heating vulcanizes it in place and thus produces a rubber and abrasive core which is integrally united with the vitrified wheel. The strength of this center core may be varied as desired within the capacity of a rubber compound of the type used. 55

60 As a further example illustrating the breadth of this invention, a resinoid bonded wheel of the softer grades may be strengthened by means of a core of a harder resinoid material. In the outer zone, one may have, for example, a mixture of 86.9% by weight of abrasive of 12 grit size and 13.1% of "Bakelite" resinoid pressed to a volume having 2.56 grams per cubic centimeter. The inner zone in such a wheel may be made of the same material but of a finer grit, such as 65 70 75

#60. The inner zone will be so proportioned and compressed as to have the same volume structure as is found in the outer zone. In this case, each will have 56% by volume of abrasive, 26% of bond and 18% of pores. For a much softer wheel, one may use the same composition for the center zone, with an outer zone having 90.2% by weight of abrasive and 9.8% of bond. One skilled in the art will know how to vary the proportions of the ingredients and to choose such methods of manufacture as will make other types of wheels as required in the industry. This invention is not limited to any particular type of wheel or method of manufacture, and various other 15 modifications of this invention will be readily apparent in view of the above disclosure.

It will, therefore, be appreciated in view of the above disclosure that we have provided a grinding wheel comprising an outer annular zone of 20 bonded abrasive material of required grinding characteristics and an inner zone integral therewith which may be made of various materials, provided they satisfy certain characteristics. These characteristics are that the inner zone 25 have such strength, ruptural deformations and modulus of elasticity as compared with the respective characteristics of the outer zone that the composite structure will be rendered capable of withstanding a higher breaking speed or possessing greater resistance to breakage due to 30 frictional heat at the wheel periphery, or both, than will a wheel of the same size made of the outer zone material. It is preferable, as above explained, that the inner zone have the higher 35 strength and ruptural deformation and that the modulus of elasticity of the two zones lie within the ratio of 1 to 2.6, but it will be appreciated that each one of these three primary characteristics may be suitably modified if the net result is one 40 of strengthening the wheel. Also, the other characteristics discussed above will be suitably controlled within the requirements of the particular wheel being manufactured. Hence, the invention claimed herein is to be interpreted as limited to the various methods, compositions and 45 structures, as well as the above defined characteristics, which are disclosed above for strengthening a grinding wheel, together with such modifications or equivalents as will be apparent to one skilled in the art.

The bonds in the two zones are deemed to be of the same class, as specified in the claims, when the bonds are both rubber compounds, or both resinoids, or both vitrified ceramic materials, etc., without regard to variations in the 55 specific proportions or compositions of the two bonds. For example, if vitrifiable ceramic mixtures are used to make the bonds of the two zones, the composition in the inner zone may be 60 materially different from that used in the outer zone, as is required to give the desired strength and other characteristics.

Having thus described the invention, what is claimed as new and desired to obtain by Letters 65 Patent is:

1. A composite grinding wheel comprising an outer annular zone of bonded granular abrasive material of required grinding characteristics and having substantially the same volume percent- 70 ages of bond, grain and pores throughout and an inner strengthening zone of bonded granular material of predetermined different characteristics which is integrally united with the outer zone, the bond and granular material of the 75 inner zone being of such compositions and pro-

portions relative to those of the outer zone that the inner zone has a higher strength than has the outer zone and such a ruptural deformation and modulus of elasticity that the composite wheel will withstand greater stress due to rotation or peripheral heat than will a wheel made wholly of the outer zone composition and structure, the ratio of the moduli of elasticity of the two zones between 1 and 2.6.

2. A grinding wheel of the type covered by 10 claim 1 in which the bond in each zone is of the same class and the granular materials and the proportions of the ingredients of the two zones are so related that the moduli of elasticity 15 of the two zones are substantially equal.

3. A composite grinding wheel of the type covered by claim 1 in which the bonded materials of the two zones are such that they have substantially equal coefficients of expansion and substantially equal drying and heat maturing 20 shrinkages whereby the two zones remain integrally united during manufacture of the wheel.

4. A composite grinding wheel as claimed in 25 claim 1 in which the bonded materials of the two zones are made of the same kind of abrasive material and bond, and the proportion of bond to abrasive in the inner zone is greater than that in the outer zone.

5. A composite grinding wheel of the type 30 covered by claim 1 in which the bonded materials of the two zones are made of the same kind of abrasive material, and the abrasive material of the inner zone contains such a considerable proportion of abrasive grains which are finer than the average size of material in the outer zone 35 that with respect to the kind and quantity of bond and the nature of the granular material in the inner zone the latter has a greater strength and ruptural deformation than has the outer zone.

6. A grinding wheel of the type covered by 40 claim 1 in which each zone is made of abrasive grains united by a vitrified ceramic material and the drying and firing shrinkages and the coefficients of expansion of the two zones are so nearly 45 alike, within the elastic limits of the zone materials, that rupture between the two zones is not caused by such shrinkages and differential contraction during manufacture of the wheel.

7. A grinding wheel of the type covered by 50 claim 1 in which the inner zone extends radially outwardly to that point at which it receives such a proportion of the stress due to rotation or peripheral heat that the wheel is materially strengthened.

8. A composite grinding wheel comprising an outer annular zone of abrasive material and bond of required grinding characteristics and having a substantially uniform structure throughout, and an inner zone formed in situ 60 of material having such a coefficient of expansion and maturing shrinkage relative to similar characteristics of the outer zone that the two zones are integrally united during manufacture, and the compositions and proportions of the materials of the two zones being such that the ratio of the moduli of elasticity of the two zones lies 65 between 1 and 2.6 and that the inner zone has a higher strength and ruptural deformation than has the outer zone, and the inner zone being of sufficient size radially as to receive such a proportion of the stress due to rotation or peripheral heat that the wheel is materially stronger than one made wholly of the outer zone composition 70 and structure.

9. A composite grinding wheel of the type covered by claim 1 in which the bond in each zone is a vitrified ceramic bond and the quantities and types of granular material and bond are so chosen with respect to the sizes of granular material used that the drying and firing shrinkages and the thermal contractions during manufacture of the wheel are so nearly equal, within the elastic limits of the materials, that rupture is not caused thereby during manufacture, and the inner zone has both a higher strength and ruptural deformation than has the outer zone.

10. A grinding wheel of uniform basic structure which has an arbor hole therethrough and which has an outer zone and a relatively narrow inner annular zone adjacent the arbor hole to which has been added a strengthening material

throughout the thickness of the wheel, the outer zone being unchanged.

11. A grinding wheel of uniform basic structure which has an arbor hole throughout and which has an outer zone and a relatively narrow inner annular zone adjacent the arbor hole impregnated throughout the thickness of the wheel with a strengthening material, the outer annular zone being unimpregnated and unchanged.

12. The grinding wheel as set forth in claim 11, in which the strengthening material is a synthetic resin.

13. The grinding wheel as set forth in claim 11, in which the strengthening material is a phenolic condensation product.

KENNETH F. WHITCOMB.  
HERBERT W. WAGNER.

5

15